

## UNITED STATES PATENT OFFICE.

FRANCIS BRADLEY AND HARRY L. FREVERT, OF PHILADELPHIA, PENNSYLVANIA.

## ARMOR PLATE AND PROCESS OF MAKING SAME.

No Drawing.

Application filed June 27, 1922. Serial No. 571,303.

*To all whom it may concern:*

Be it known that we, FRANCIS BRADLEY and HARRY L. FREVERT, citizens of the United States, residing at Philadelphia, county of

5 Philadelphia, and State of Pennsylvania, have invented a new and useful Improvement in Armor Plates and Processes of Making Same, of which the following is a full, clear, and exact description, reference being 10 had to the accompanying drawings, which form a part of this specification.

In an application filed by us June 27, 1922, Serial No. 571,301, we set forth the discovery that if armor plate which is already 15 treated, by known methods, to produce a plate having a hardened front with a carburized face and a tough back, is drawn at a temperature above 500° F. and below 1100° F., so as to remove from the hard front 20 practically all the brittleness and a large portion of the hardness, while maintaining the stiffness required to offer extraordinary resistance to displacement, it will offer greater resistance to penetration, with proj- 25 ectiles of the present improved type, than is offered by a plate of the ordinary type, wherein the hard front of the plate is unable to break the point of the projectile and is itself cracked and spalled off with less expenditure of power than would be required 30 were the metal to remain in position and offer great resistance to displacement.

The object of the present invention is to 35 still further increase the resistance of the plate to perforation and at the same time prevent cracking under the shock of impact.

A hard faced tough backed plate of the 40 type to which our invention is applicable may be produced, for example, by the following process, well known to those skilled in the art: An ingot of any suitable composition is cast, and after reheating is forged or rolled into a plate of a thickness about 45 20% in excess of the thickness desired for the finished plate. The plate, thus formed, may be reheated and annealed, or reheated to below the critical temperature and cooled either quickly or slowly. The side of the 50 plate intended for the face is then cleaned of all scale and a brick container built around its edges. The container is filled with a suitable carburizing compound, and a similar plate is laid face down upon it, the 55 pair of plates being then heated to a tem-

perature and for a time suitable for penetration of carbon into the face of the plate to the desired depth and extent, or the plate may be carburized by a gas.

After the carburization of the plate, by 60 the absorption thereby of the desired carbon, the plate is carefully cooled, and freed of scale, the face protected by a carbonaceous covering, reheated to a very low forging temperature and forged to final thickness. The plate is then reheated to a tem- 65 perature considerably above its critical tem- perature, quenched, again reheated, but to a less degree than before and again quenched. The plate is then again reheated to a point 70 below its critical temperature, bent and cooled slowly; again reheated to a point well below its critical temperature and quenched. The face of the plate is then heated rapidly to well above its critical temperature, while 75 the back is kept below that temperature and the plate quenched throughout. In this heating operation, the temperature of the plate is raised to above the critical tempera- 80 ture to a depth substantially exceeding the relatively thin carburized face zone and it is this part of the plate, which includes the carburized face and a zone to the rear thereof, which we call the "front."

In the above described, and other well 85 known processes of face hardening armor plate, it is present practice to harden to a depth, in the case (say) of a 13 $\frac{1}{2}$  inch plate, of substantially less than five inches to not over about six inches or from thirty-five to 90 less than forty-five per cent. of the thickness of the plate. Increase of the hardened zone, in the case of plates of the present type, would not only not give greater resistance to 95 penetration, but would be detrimental, as it would provide a disproportionately thin tough back. In manufacturing our improved armor plate, however, we find that if the plate (say 13 $\frac{1}{2}$  inches in thickness) is hardened to a depth varying from substan- 100 tially over six inches to nearly nine inches, or from at least forty-five per cent. to about sixty-five per cent. of the thickness of the plate, and is then drawn at a temperature of from 500 to 1100 degrees F. (preferably 650 105 degrees F.), the resistance of the plate to perforation will be still further increased, while, by reason of the removal of the brittleness and a large portion of the hardness from the initially hardened plate, the tough 110

or ductile zone at the back is sufficiently thick to prevent cracking of the plate under shock of impact.

In producing initially the plate having a hard front and a tough back, the plate may be carburized to the depth of (preferably) from seven to ten per cent. of the thickness of the plate. Such initial face carburization is preferable in the case of most plates and where expense is not an important factor; but the benefits and advantages of our invention, to a substantial degree, are secured without initial face carburization. Our plates may therefore have a substantially uniform carbon content.

It is not intended to limit the present invention to face carburization, but to claim the invention broadly whether or not the plate is face carburized and also to claim the more specific invention wherein the plate is of substantially uniform carbon content. In an application filed of even date herewith, Serial No. 571,302, we have described and claimed an invention having the same essential features as those herein set forth but restricted to face carburization of the plate, such invention being both a specific modification of the present invention and an embodiment of and improvement upon the application filed by us of even date herewith, Serial No. 571,301.

This application is a continuation in part of application Serial No. 505,889, filed October 6, 1921.

Having now fully described our invention, what we claim and desire to protect by Letters Patent is—

1. The process of so treating armor plate as to render it resistant to perforation, which comprises treating the plate to produce a

tough back and a front hardened to a depth of from forty-five to sixty-five per cent. of the thickness of the plate, and then drawing the plate at a temperature not below 500 degrees F. nor above 1100 degrees F. 45

2. The process of producing armor plate so as to render it resistant to perforation, which comprises treating a plate of substantially uniform carbon content to produce a tough back and a front hardened to a depth of from forty-five to sixty-five per cent. of the thickness of the plate while maintaining the uniform carbon content of the plate, and then drawing the plate at a temperature not below 500 degrees F. nor above 1100 degrees F. 50 55

3. As a new article of manufacture, an armor plate provided with a tough back and a stiff hardened front from which the normal brittleness has been substantially removed and whose normal hardness has been substantially diminished, the depth of the de-brittled, stiff zone of reduced hardness being from forty-five to sixty-five per cent. 60 65 of the thickness of the plate. 65

4. As a new article of manufacture, an armor plate of substantially uniform carbon content provided with a tough back and a stiff hardened front from which the normal brittleness has been substantially removed and whose normal hardness has been substantially diminished, the depth of the de-brittled, stiff zone of reduced hardness being from forty-five per cent. to sixty-five per cent. of the thickness of the plate. 70 75

In testimony of which invention, we have hereunto set our hands, at Philada., Penna., on this 21st day of June, 1922.

FRANCIS BRADLEY.  
HARRY L. FREVERT.